

# UNITED STATES PATENT OFFICE.

WILLIAM P. TAGGART, OF READING, PENNSYLVANIA, ASSIGNOR TO THE ZWOYER FUEL COMPANY, OF NEW JERSEY.

## PROCESS OF PRODUCING ARTIFICIAL FUEL.

SPECIFICATION forming part of Letters Patent No. 655,282, dated August 7, 1900.

Application filed May 18, 1900. Serial No. 17,157. (No specimens.)

*To all whom it may concern:*

Be it known that I, WILLIAM P. TAGGART, a citizen of the United States, and a resident of Reading, in the county of Berks and State 5 of Pennsylvania, have invented a certain new and useful Improvement in Artificial Fuels and the Processes for the Production of the Same, of which the following is a specification.

The purpose of my invention is to utilize 10 the vast heaps of comminuted coal or culm which have accumulated at every worked coal mine in this country and which are now a waste product by forming the same into compact, durable, waterproof lumps of convenient size for practical use as a fuel.

I am aware that many attempts have heretofore been made to accomplish this result, but owing either to defects in the product or in the process involved or because the cost of 15 production was such as to preclude competition with the natural fuel none of these prior attempts have proved commercially successful, and comminuted coal still continues to be a waste product. My invention is intended to overcome these difficulties and produces a fuel not only considerably cheaper, but in many respects superior to the natural product. A common defect of these prior processes has been that the importance of having 20 the particles of coal to be treated of small and practically uniform size has not been recognized. Dust and particles as large and larger than a pea have been combined indiscriminately into one lump. In consequence either the attachment of the binder to these 25 larger particles is feeble and the resulting lump is friable or so large a quantity of binder is required as to render the cost of production prohibitory. Furthermore, no matter how much binder is used the difficulty is not overcome, since these artificial fuels are all 30 molded into geometrical forms under heavy pressure. Thus the larger particles are crushed, and when so crushed there is no binder at all between the resulting particles to hold them together. The consequence is 35 that the product is friable and the waste incident to transportation and handling is so great as to render the residue of the fuel too 40 expensive for use as compared with the natural product.

My process consists in first reducing the culm to be treated to particles of small and uniform size, the finer the better. Economy of production is of the first importance in every commercial manufacture on a large scale. For this reason in actual practice I do not reduce my culm to a powder, but screen it through a No. 12 screen, using everything which will pass the screen and excluding everything which 55 will not. This gives a good practical result, and, all things considered, is what I prefer. While a coarser screen may be used, and thus some crushing of larger particles be dispensed with, which is of course an economy, it will be 60 at the expense of the quality of the product, and in this specification and in its claims when I speak of "particles of culm of small and uniform size" I desire to be understood as meaning and including all particles which will pass 65 through a No. 12 screen, including of course a slight margin of difference on the coarser side. The culm in this condition of subdivision is then introduced into a mixer, and intimately mixed with a binding solution 70 which consists of from five to six pounds of dextrine and five pounds of salt dissolved in twelve gallons of water to each ton of culm. After the culm is intimately mixed with the binding solution it appears to be slightly 75 moist and is slightly cohesive. It is then subjected to strong pressure in molds of any desired geometric form, which compacts the contents of the mold, bringing the particles into such close contact with one another that 80 a relatively-small quantity of binder suffices to unite them into a firmly coherent lump. The molded lumps are then baked at a heat 85 of, say, 300° to 600° Fahrenheit in an oven until perfectly dry and hard, when the particles of culm will be found to cohere firmly to one another, and each molded lump will have become a compact, coherent, and non-friable entity. Lastly, and while still hot from the drying oven, the molded lumps are 90 passed through a waterproofing bath. This bath may consist of any waterproof mixture or material which is combustible and remains liquid at a temperature somewhat lower than the temperature of the fuel lumps when introduced into the bath, which dries readily 95 and when dry is not sticky and is reasonably 100

tough. For this purpose I have found a bath composed of melted rosin and crude petroleum in the proportion of twenty-four and three-fourth pounds of melted rosin to one-half gallon of crude petroleum to answer very well, and this is about the consumption of waterproofing material I expect to use for each ton of culm. The addition of two to three pounds of paraffin - wax improves the bath somewhat, but increases its cost. This bath is of course used in a fluid condition, and the result to be aimed at in its use is not to make a superficial glaze which might chip off, but to induce the waterproofing mixture to penetrate somewhat below the surface, so that while it protects the fuel lumps from moisture it is itself protected from harmful abrasion by the exposed surface of the fuel lump. If the fuel is surely to be used where made and soon after it is made and kept under cover until used, the waterproofing process may be dispensed with; but unless this is certain the fuel should be waterproofed when made.

25 The result of my process is a cleanly compact non-friable waterproof fuel which ignites readily, burns with considerable clear and smokeless flame, and leaves a very little clean ash as a residue. A fire made from it requires a minimum of attention, since the fuel retains its original form until practically quite consumed and does not clinker or run together so as to clog the draft. Also it makes a very lasting fire. An ordinary grate full of my fuel kindled one day will on the following day still hold fire sufficient to ignite a fresh charge of fuel without the use of any wood or other kindling. My experiments lead me to believe that pound for pound my fuel will yield more heat than the coal from which it is made in its natural state, a result I attribute to the thoroughness with which it is consumed, as it leaves practically nothing combustible which is not wholly burned.

While I do not intend to limit myself to the exact proportions hereinbefore given, since it is obvious that they may be departed from to some extent without seriously impairing the result, still my experiments indicate that those proportions are certainly good, and probably the best.

Having thus described my invention, what I claim as new, and desire to secure by Letters Patent, is—

1. The within-described process of making artificial fuel, which consists in mixing particles of coal reduced to small and substantially uniform size with a solution of dextrine and salt, pressing this mixture into lumps of any desired form and size, and then baking the same until thoroughly dry and hard.

2. The within-described process of making artificial fuel, which consists in mixing particles of coal reduced to small and substantially uniform size with a solution of dextrine and salt, pressing this mixture into lumps of any desired form and size, baking them until thoroughly dry and hard, and passing the same through a waterproofing bath.

3. As a new article of manufacture, an artificial fuel composed of particles of coal reduced to small and substantially uniform size bound together by dextrine and salt, and pressed into a geometrical form.

4. As a new article of manufacture, an artificial fuel composed of particles of coal reduced to small and substantially uniform size bound together by dextrine and salt, and pressed into a geometrical form, and provided with a waterproof coating.

Signed at the city of New York, in the county of New York and State of New York, this 8th day of May, A. D. 1900.

W. P. TAGGART.

Witnesses:

F. M. DONSBACH,  
WM. O'SHAUGHNESSY.